

## UNITED STATES PATENT OFFICE

2,070,268

## DIELECTRIC MEDIUM

Hugh Bryson Glass, Anniston, Ala., assignor to  
Swann Research, Incorporated, a corporation  
of Alabama

No Drawing. Application July 10, 1931, Serial  
No. 550,047

2 Claims. (Cl. 252—1)

This invention relates to new compounds having improved dielectric and insulating properties. One object of this invention is the provision of means whereby the physical and electrical properties of chlorinated diaryl compositions may be changed at will within certain limits. Another object is the production of an improved dielectric medium adapted for use in electrical devices such as condensers or capacitors.

10 In the design of electrical condensers or capacitors for various purposes such as radio, alternating current motor and various other uses, it is particularly advantageous, in order to confine the apparatus in as small a space as possible to use as an impregnant a dielectric having as high a dielectric constant as practicable.

Condensers or capacitors usually consist of alternate layers of conducting and non-conducting material, the latter usually being paper. Alternate conducting plates during operation are charged to a difference of electrical potential and are connected to separate terminals. The pack when suitably supported is subjected to drying and impregnating treatment with a dielectric and insulating oil. For this purpose certain of the chlorinated diphenyl oils have already been proposed. In particular, chlorinated diphenyl oils containing from 42 to 54% of chlorine have been found useful for this purpose, these products possessing a fairly good dielectric constant and low power factor and high electrical resistivity.

I have now discovered that the capacity of electrical devices such as condensers can be materially improved by the use of certain chlorinated high boiling diaryl compounds either alone or admixed with chlorinated diphenyl. The high boiling compounds which I prefer to employ are produced as a by-product during the thermal synthesis of diphenyl from benzol. I have also discovered that the density of the resulting chlorinated product containing the high boiling compounds is appreciably lower than that of the chlorinated diphenyl itself, the lower density being advantageous in decreasing the weight of the material utilized and hence the weight of the finished condenser.

The composition obtained by my invention may also be used alone or together with other ingredients as a cooling medium for transformers, switches and other electrical devices where insulating oils are commonly used, and which have elements charged during operation to a difference of electrical potential.

55 The high boiling compounds which I employ

in the production of my improved composition are rather difficult to identify chemically. They are, as far as is now known, mainly composed of the hydrocarbons, ortho and para diphenyl benzene and hence are related chemically and structurally to diphenyl. The origin of these hydrocarbons is similar to that of diphenyl, i. e., they are produced by the pyrolysis of benzol and are separated from the pyrolysis product by distillation.

10 Due to the appreciably higher boiling point possessed by these bodies over that of diphenyl itself it is customary, when making a separation of the pyrolysis product obtained from benzene, to distill off a technical diphenyl fraction between 15 temperatures of 250. to 270° C., at atmospheric pressure. The residue or high boiling compounds remaining behind in the distillation flask may be employed as such for the practice of this invention, however, it is desirable to further distill 20 these high boiling compounds. In doing so the temperature may be raised to 390 to 400° C., and the high boiling fraction is thus divided into two parts and known as "distilled high boiling compounds" and "still bottoms". The last fraction 25 or "still bottoms" thus obtained consists of some very high boiling compounds together with tar and carbon.

30 In the preparation of my improved dielectric I prefer to mix together varying proportions of diphenyl together with the distilled high boiling compounds obtained as above and chlorinate the mixture by passing in chlorine gas. Rapid and efficient chlorination can be effected by the addition of a small amount of iron or iron chloride to the mixture of hydrocarbons.

35 When the chlorination has reached the desired degree the product is distilled preferably in vacua until it has almost completely distilled over. Yields on distillation in the neighborhood of 95% 40 may be expected. Considerable benefit is obtained by the addition of small amounts of lime to the distilling flask, which addition serves to prevent traces of iron chloride or hydrochloric acid from coming over during distillation, thus 45 yielding a lighter colored product of considerably better electrical resistivity.

In the application of my invention to metallic foil condensers I may build the pack of alternate sheets of metallic foil and paper. The pack is 50 then carefully dried preferably in a vacuum and while still hot and in the vacuum impregnator my improved dielectric insulating liquid is admitted. Penetration of the dielectric liquid into the interior of the pack may be aided somewhat by 55

the application of pressure on the liquid impregnant after sufficient time has been given to expell most of the air by the vacuum treatment. By choosing a composition of suitable viscosity and correctly determining the time of impregnation by trial a satisfactory uniform penetration may be had.

10 The composition and properties of my new composition are illustrated in the following Table 10 I. By way of comparison the properties of two samples of chlorinated diphenyl are included in this table.

Table I

| 15 | Hydrocarbon compositions           |                                  | Properties of dielectric |                                   |                                |                                                 |
|----|------------------------------------|----------------------------------|--------------------------|-----------------------------------|--------------------------------|-------------------------------------------------|
|    | Diphenyl                           | Distilled high boiling compounds | Chlorine content         | Viscosity sec. Saybolt at 210° F. | Specific gravity at 65°/65° C. | Dielectric constant K at 100° C. (1,000 cycles) |
| 20 | Percent                            | Percent                          | Percent                  |                                   |                                |                                                 |
| 1  | 0                                  | 100                              | 23.9                     | 63                                | 1.251                          | 4.35                                            |
| 2  | 0                                  | 100                              | 40.3                     | 290                               | 1.405                          | 4.98                                            |
| 3  | 80                                 | 20                               | 41.2                     | 35.7                              | 1.352                          | 4.87                                            |
| 4  | 80                                 | 20                               | 52.2                     | 47.5                              | 1.400                          | 4.56                                            |
| 5  | 50                                 | 50                               | 42.0                     | 48.8                              | 1.383                          | 4.84                                            |
| 6  | 50                                 | 50                               | 36.4                     | 40.8                              | 1.324                          | 4.89                                            |
| 30 | Properties of chlorinated diphenyl |                                  |                          |                                   |                                |                                                 |
| 7  | 100                                | 0                                | 54.0                     | 46.0                              | 1.523                          | 4.30                                            |
| 8  | 100                                | 0                                | 42.0                     | 34.0                              | 1.380                          | 4.80                                            |

35 The possibilities of the invention will be apparent from the above table.

Among other things it will be apparent that if a dielectric of low specific gravity is desired it is preferable to use the distilled high boiling compounds without admixture of diphenyl.

40 By comparing compositions 1 and 7 in the above table it will be seen that in this manner a decrease of 17.8% in specific gravity is obtained without a sacrifice in the dielectric properties.

45 If 20% of distilled high boiling compounds is

admixed with 80% of diphenyl and the mixture chlorinated to a viscosity of 47.5 seconds, the dielectric constant of the distilled product will have increased 0.26 unit over that of diphenyl, an increase of over 6%. Compare compositions 5 4 and 7. If 50% of distilled high boiling compounds be admixed with 50% of diphenyl and the mixture chlorinated to a viscosity of 48.8 seconds, the dielectric constant will be over 12% greater than that possessed by chlorinated diphenyl of similar viscosity.

10 It will be appreciated that variation in the several properties of these compositions is of importance for in some applications it will be found that viscosity of the material is of importance, 15 in others that density is important, and in others that the dielectric constant is important.

While I have described my invention in several forms, it will be obvious to those skilled in the art that it is not so limited, but is susceptible of 20 various other changes and modifications without departing from the spirit thereof, and I desire, therefore, that only such limitations shall be placed thereupon as are imposed by the prior art or as are specifically set forth in the appended 25 claims.

What I claim is:

1. A dielectric medium comprising a chlorinated mixture of diphenyl and complex hydrocarbons having a higher boiling point than diphenyl, and produced in the pyrolysis of benzol, 30 said mixture having a chlorine content up to 52.2% and the proportion of complex hydrocarbons therein to diphenyl varying from 20% to 100%.

2. A dielectric medium comprising chlorinated complex hydrocarbons mixed with chlorinated diphenyl, said complex hydrocarbons having a boiling point above that of diphenyl and having been produced by the pyrolysis of benzol, said 40 chlorinated mixture of hydrocarbons and diphenyl containing up to 50% of chlorinated diphenyl, and the chlorinated mixture having a Saybolt viscosity between 40 and 290 seconds at 210° F.

HUGH BRYSON GLASS. 45